

## UNITED STATES PATENT OFFICE

EARL C. SMITH, OF CANTON, OHIO, ASSIGNOR TO REPUBLIC STEEL CORPORATION, OF YOUNGSTOWN, OHIO, A CORPORATION OF NEW JERSEY

## METHOD OF CASTING METAL

No Drawing.

Application filed November 26, 1927. Serial No. 236,006.

The present invention relates broadly to the art of metal founding and more particularly to an improved method having a special value with reference to the casting of relatively large bodies of a more or less solid nature or having sections of substantial cross sectional area, such, for example, as those present in ingots.

It is well recognized in the art to which the invention relates that at least a large part of the difficulty in the casting of ingots arises from the manner in which the molten metal solidifies or freezes. Ordinary dead melted steel freezes at a rate substantially proportionate to the square root of the time in minutes. In other words, the first inch freezes in approximately a minute, two inches in approximately 4 minutes, 5 inches in approximately 25 minutes, etc. It will thus be seen that a 30 inch ingot requires substantially 225 minutes to freeze to the center. In actual practice the outer shell freezes very quickly and the inner liquid portion tends to tear itself to pieces during freezing, due to shrinkage. If the rate of freezing could be accelerated in the inner portion of the ingot, this danger of tearing to pieces would be minimized and no difficulty would be encountered. The present invention has for one of its objects the controlling of the freezing so as to eliminate difficulties with respect to shrinkage, preferably by insuring freezing of the lower portion of the ingot before the sink head is out of action, whereby there is no efficient filling of any shrinkage cavities.

In the pouring of most ingots, it is necessary to pour at temperatures high enough to insure fluidity and to take care of certain reactions. In order to secure the desired condition it is customary to err on the side of too high a temperature so that the furnace operator usually delivers metal into the ladle at too high a temperature, and this is in turn poured into the molds with this extra temperature. In accordance with the present

invention, I preferably add to the metal either immediately prior to the pouring or during the pouring a material or materials which will boil off at the temperatures present. Such materials must necessarily be of a more or less volatile character, having a boiling point below the temperature of the metal being cast in order to insure volatilization. The heat of vaporization of such added materials, either metallic or non-metallic, is usually very high and advantage can be taken of the heat absorption thereof to enable the cooling of the interior of the ingot during pouring and freezing to be satisfactorily controlled.

In accordance with the present invention, I preferably add to the metal, either immediately prior to or during the pouring operation, a volatile material such as lead, fluorides, or other materials, characterized by this boiling action, and take advantage of the heat absorption thereof to increase the rate of cooling of the interior of the ingot.

By the use of the present invention, the production of castings, such as ingots, having a more uniform and desirable texture is insured and the rate of solidification is hastened. The materials added, due to their volatile nature at the temperatures present, do not interfere with the obtaining of the desired characteristics in the finished product. The invention is obviously not limited to any specific castings or materials, and is important not only with dead melted steels, but with open steel ingots after pouring.

I claim:

1. In the method of forming metal castings, the step comprising adding to the interior of the casting while in molten condition an artificial refrigerator in the form of a solid material having a high heat of vaporization and volatilizable at the temperature of the metal from which the casting is to be made, and utilizing the heat absorption of

such material during volatilization to hasten the cooling of the interior of the casting.

2. In the art of casting metal ingots, the method which consists in adding to the metal while in a molten state a solid volatile material having a boiling point below the temperature of the molten metal and permitting such added material to reach a state of volatilization, the said volatile material functioning during the process of volatilization to extract heat from the interior of the ingot and expedite the cooling action thereof.

10 In testimony whereof I have hereunto set my hand.

15

**EARL C. SMITH.**

20

25

30

35

40

45

50

55

60

65